# EUROPEAN PATENT SPECIFICATION

(11) **EP 1 130 460 B1**
(45) Date of publication and mention of the grant of the patent: **06.06.2007**
(21) Application number: 01200764.7
(22) Date of filing: 01.03.2001
(51) Int. Cl.: G03C 1/79, D21H 23/30, D21H 23/46

(54) **Process for the preparation of polymer laminated base paper and polymer laminated photographic base paper obtainable by said process**
Verfahren zur Herstellung polymerlaminierter Papierträger und durch dieses Verfahren hergestellte polymerlaminierte photographische Papierträger
Procédé de préparation de papier de support recouvert de polymère et papier de support photographique recouvert de polymère obtenu par ce procédé

(30) Priority: 03.03.2000 EP 00200764
(43) Date of publication of application: 05.09.2001
(73) Proprietor: Fuji Photo Film B.V., 5047 TK Tilburg (NL)
(72) Inventor: Bouwstra, Jan Bastiaan, 3721 AJ Bilthoven (NL); de Vries, Ieke, 5171 WV Kaatsheuvel (NL)
(74) Representative: Prins, Adrianus Willem

(56) References cited:
- EP-A- 0 573 753
- EP-A- 0 704 753
- EP-A- 0 952 483
- DE-A- 19 821 446
- JP-A- 57 102 622
- US-A- 5 182 161
- US-A- 6 030 742

## Description

The invention is directed to the preparation of polymer laminated base paper and more in particular to the preparation of polymer laminated photographic base paper.

Polymer laminated base paper for photographic printing paper is conventionally prepared from a base paper that is laminated with at least one polymer resin layer, usually a titanium dioxide filled polyethylene, polypropylene or a polymethylene-methacrylate resin, by extrusion-coating (or co-extrusion-coating) of a polymer melt onto the surface of the base paper.

EP-A-0 704 753 describes pretreatment of a paper base with corona discharge treatment and flame treatment.

In JP-A 57-102622 a process is described for the extrusion-coating of a base paper with polyethylene, in which process the base paper is subjected to a corona treatment, followed by heating to a temperature of at least 80°C. This process aims at improving the adhesion between base paper and polymer coating.

An important aspect of the quality of polymer resin laminated base paper is the resin surface appearance, which should not have a large number of crater-like defects (or pits) after extrusion-coating of the polymer resin on the base paper.

Further important aspects of photographic base paper are the speed of production and the thickness of the polymer layers. Both aspects are important in view of the economy of the process of producing photographic print paper. The formation of pits has turned out to be strongly dependent on those aspects.

It has been attempted to suppress the number of pits by increasing the thickness of the polymer resin layer. At high extrusion-coating speeds, such as over 300 m/min this is not sufficiently effective, unless very large amounts of polymer are used. Furthermore, it has economical disadvantages as the polymer resin is an important cost factor in the production of photographic print paper.

At extrusion-coating speeds of the polymer resin of 300 m/min or more it has been found to be much more difficult to reduce the number of pits.

In the art of providing polymer laminated photographic base paper there is a need for high speed production, especially during the extrusion-coating of the paper with the polymer resin, whereby the amount of pits remains at a sufficiently low value.

Accordingly it is an object of the present invention to provide a process for the preparation of a polymer laminated base paper, more in particular a polymer laminated photographic base paper, wherein the number of pits is decreased, especially at higher extrusion-coating speeds.

It is a further object of the invention to provide a process for the preparation of a polymer laminated base paper, more in particular a polymer laminated photographic base paper, wherein the number of pits is decreased, at higher extrusion-coating speeds, without the need to increase the polymer weight.

The present invention is based thereon, that the coated paper shows less pits in case the base paper web is heated, preferably by infrared radiation, prior to the extrusion-coating with the polymer resin.

Accordingly the present invention is directed to a process for the preparation of polymer laminated base paper, said process comprising laminating a base paper web on at least one side thereof with at least one polymer layer, by extrusion-coating at a coating speed of 300 m/min or more, wherein the said base paper web is heated prior to laminating.

Surprisingly it has been found that with this process the number of pits can be reduced, even at high extrusion- coating speeds, such as extrusion-coating speeds in excess of 300m/min. The advantages of the invention become apparent already at extrusion speeds of 300 m/min or over. It is preferred to use a speed of at least 350 m/min, more in particular at least 400 m/min. Presently an upper limit of 700 m/min is considered acceptable.

In the broadest sense the present invention resides therein that the paper web is heated just prior to the (co-)extrusion-coating. This heating can be done by the application of heated air, heated rollers and/or by radiation. More in particular, preference is given to the use of radiation in the Near Infra Red (NIR) region. In particular, it is to be noted that the NIR radiation can be emitted at radiation temperatures of over 2500 K, preferably over 2900 K, most preferred over 3000 K. Generally, the upper limit for the emission temperature is 3500 K.

It has been found that surprisingly the use of NIR radiation provides good results in terms of product properties. Further, it has been found that in terms of heating rate the use of NIR has advantages.

The advantages of the treatment of the web by infra-red radiation, with wavelength ranges between 0.8 µm and 1 mm, results in the increase of the web temperature in an extremely short treatment period, usually less than 1 second. With the use of conventional heating technologies this is less easy too achieve. The fastest temperature increase can be realised with NIR radiation of a wavelength between 0.8 and 1.5 µm. Advantages of this method are that it is contactless, eliminating the risk of mechanical damage as in case of the use of heated rollers and is highly flexible as the heating power can continuously and immediately be adapted to process needs, such as varying laminating speed, with temperature controlling devices which control the surface temperature.

In the heating step prior to the extrusion-coating the temperature of the paper is preferably raised to a value of at least 30°C, preferably to a value between 30 and 125°C. More in particular the upper limit of the temperature of the web is 90°C. In case energy consumption is a consideration, the temperature may be kept at a value of less than 80°C without negative effects.

The extrusion-coating can be done with one layer of polymer or with a combination of polymer layers by co-extrusion. The paper web can be coated on one side or on both sides, the latter embodiment having preference. The polymers to be used for the extrusion-coating are the conventional polymers used in paper coating, more in particular in the preparation of photographic base paper. Examples are polyolefins, polyacrylates or polyesters. More in particular, the coating is done using low-density polyethylene, high density polyethylene and blends thereof. The amount of polymer coating depends on the required properties of the laminated base paper, such as stiffness, gloss, number of pits and the like. More in particular the amount is preferably not more than 50 g/m², more preferably between 25 and 50 g/m².

The heating step can be incorporated in an extrusion-coating line for paper. It is to be noted that in case of the use of more than one layer of polymer resin it is possible to use co-extrusion. The term 'extrusion' is therefor intended to include also co-extrusion.

In the extrusion line also other treatments of the paper web can be used such as corona treatment, ozone treatment, flame-treatment and plasma treatment, which treatments all aim at improving the adhesion of the polymer melt to the base paper web.

The invention is now elucidated on the basis of the attached figure. In this figure an extrusion-coating line has been shown. The base-paper web is fed, via a number of rollers, past a corona treatment, via the nip-roll to the nip-zone. The polymer melt and the base paper web come together in the nip. The polymer melt is then cooled on the chill-roll and is released from the chill-roll at the release-roll, from where it is transported further.

Between the corona treatment and the nip-roll, NIR radiation equipment is installed. In order to get a very good efficiency, the infra-red radiation is provided from one side and a radiation mirror is provided on the other side. It is also possible to install the NIR-radiation equipment before the corona treatment.

It is to be noted that the present figure shows lamination on only one side of the paper web. In case lamination on both sides has to be provided, the partly laminated paper web can be laminated on the other side in a comparable co-extrusion line. It is also possible to include a second extruder and, if necessary, suitable radiation equipment in this line.

The invention is now elucidated on the basis of the Example.

### Example

Two paper substrates were used for testing. These substrates, or base papers, represent a range of base paper qualities as can be found in the market. Paper substrate '1' represents a good quality in relation to the number of pits. Paper substrate '2' represents a lower quality.

The web width of the substrates was 47 cm. The substrates were first extrusion coated with 21.0 g/m2 transparent polyolefin resin film on the backside at a line speed of 200 m/min.

Before extrusion-coating of the topside, the substrate was pretreated with corona and subsequently preheated with NIR radiation up to a temperature of 39°C or 83°C. The treating width of the NIR-equipment covered 24 cm in the centre of the total web width of 47 cm. For the pretreatment two NIR-units were used. After the online pretreatments (Corona and preheating) the substrate was extrusion coated at the topside with a polyolefin resin LDPE of 28 g/m2 (containing metaloxide, dyes, coloured pigments, optical brighteners and the like) at a speed of 400 m/min. The hotmelt (temperature 326°C) was nipped (pressure 6 bar) between the substrate and a cooling chill-roll. Because of the NIR-pretreatment the crater like defects or so-called pits defects decreased in comparison to the samples which received no heat pretreatment (remaining at room temperature). The NIR-pretreatment shows no disadvantage in the number of releasing defects, when the extrusion coated web releases from the cooling chill-roll.

The following test results are obtained which shows the effectivity of the heat pretreatment in order to reduce the number of pits defects:

| | Paper type 1 | | Paper type 2 | |
|---|---|---|---|---|
| | Number of pits per 4mm² | | Number of pits per 4mm² | |
| | (800-1200 µm²) | (>1200 µm²) | (800-1200 µm²) | (>1200 µm²) |
| No NIR treatment(23°C) | 9.3 | 2.3 | 22.3 | 9.3 |
| NIR treatment (39°C) | 1.7 | 0.3 | 14.3 | 5.0 |
| NIR treatment (83°C) | 2.0 | 1.3 | 9.7 | 1.3 |

In the example the following methods were used to determine the various parameters:
Pits: Olympus microscope; measure area of 4 mm²
Web temperature: Minolta Land temperature meter.

These results show that for the lower quality base paper type, a significant reduction of the number of pits can be realised, even at temperatures as high as 83°C. With a good quality of base paper also a significant reduction of the number of pits is realised.

## Claims

1. Process for the preparation of polymer laminated base paper, said process comprising laminating a base paper web on at least one side thereof with at least one polymer layer by extrusion-coating at a coating speed of 300 m/min or more, wherein the said base paper web is heated prior to laminating, wherein said heating is done by use of near-infrared radiation.

2. Process according to claim 1, wherein the coating speed is at least 350, preferably at least 400 m/min, more in particular not more than 700 m/min.

3. Process according to claim 1 or 2, wherein the said infrared radiation is emitted at temperatures of over 2500 K.

4. Process according to claims 1-3, wherein the base paper web is extrusion-coated on both sides.

5. Process according to claims 1-4, wherein the said polymer is a polyolefin, a polyacrylate or a polyester.

6. Process according to claims 1-5, wherein the said base paper web is preheated to a temperature of between 30 and 125°C.

7. Process according to claim 6, wherein the temperature is not more than 90°C.

8. Process according to claims 1-7, wherein the base paper web is subjected to one or more additional other treatments, prior to extrusion-coating.

9. Process according to claim 8, wherein the said other treatment comprises at least one of corona treatment, ozone treatment, flame treatment and plasma treatment.

10. Process according to claims 1-9, wherein the laminated base paper is a polymer laminated photographic base paper.

11. Process according to claim 10, wherein the polymer laminated photographic base paper is provided with at least one layer of a photographic emulsion.

12. Process according to claim 11, wherein the polymer laminated photographic base paper is provided with at least one layer of a gelatin sublayer between the polymer coating and the photographic emulsion.

13. Polymer laminated photographic base paper or print paper, comprising a base paper web on at least one side thereof a polymer coating in an amount of between 25 and 50 g/m², which laminated paper is obtainable by the process of claim 10-12.

## Patentansprüche

1. Verfahren zur Herstellung von polymerlaminierten Rohpapier (base paper), wobei das Verfahren das Laminieren einer Rohpapierbahn auf wenigstens einer Seite dieser mit wenigstens einer Polymerschicht durch Extrusionsbeschichtung mit einer Beschichtungsgeschwindigkeit von 300 m/Min. oder mehr umfasst, wobei die Rohpapierbahn vor dem Laminieren erwärmt wird, wobei die Erwärmung unter Verwendung einer nahen Infrarotstrahlung durchgeführt wird.

2. Verfahren nach Anspruch 1, wobei die Beschichtungsgeschwindigkeit wenigstens 350, vorzugsweise wenigstens 400 m/Min, und insbesondere nicht mehr als 700 m/Min. beträgt.

3. Verfahren nach Anspruch 1 oder 2, wobei die Infrarotstrahlung bei Temperaturen von über 2.500 K emittiert wird.

4. Verfahren nach den Ansprüchen 1 - 3, wobei die Rohpapierbahn auf beiden Seiten extrusionsbeschichtet wird.

5. Verfahren nach den Ansprüchen 1 - 4, wobei das Polymer ein Polyolefin, ein Polyacrylat oder ein Polyester ist.

6. Verfahren nach den Ansprüchen 1 - 5, wobei die Rohpapierbahn auf eine Temperatur von zwischen 30 bis 125 °C vorgewärmt wird.

7. Verfahren nach Anspruch 6, wobei die Temperatur nicht mehr als 90 °C beträgt.

8. Verfahren nach den Ansprüchen 1 - 7, wobei die Rohpapierbahn vor der Extrusionsbeschichtung einer oder mehreren zusätzlichen anderen Behandlungen unterworfen wird.

9. Verfahren nach Anspruch 8, wobei diese andere Behandlung wenigstens eine aus einer Koronabehandlung, einer Ozonbehandlung, einer Flammenbehandlung und einer Plasmabehandlung umfasst.

10. Verfahren nach den Ansprüchen 1 - 9, wobei das laminierte Rohpapier ein polymerlaminiertes fotografisches Rohpapier ist.

11. Verfahren nach Anspruch 10, wobei das polymerlaminierte fotografische Rohpapier mit wenigstens einer Schicht einer fotografischen Emulsion versehen wird.

12. Verfahren nach Anspruch 11, wobei das polymerlaminierte fotografische Rohpapier mit wenigstens einer Schicht aus einer Gelatineunterschicht zwischen der Polymerschicht und der fotografischen Emulsion versehen wird.

13. Polymerlaminiertes fotografisches Rohpapier oder Druckpapier umfassend eine Rohpapierbahn, auf wenigstens einer Seite dieser eine Polymerbeschichtung in einer Menge von zwischen 25 und 50 g/m², wobei das laminierte Papier durch das Verfahren der Ansprüche 10 -12 erhaltbar ist.

## Revendications

1. Procédé pour la préparation de papier à base de stratifié de polymère, ledit procédé comprenant la stratification d'une feuille continue de papier de base sur au moins un côté de celle-ci avec au moins une couche de polymère par revêtement par extrusion à une vitesse de revêtement de 300 m/min ou plus, dans lequel ladite feuille continue de papier de base est chauffée avant stratification, et dans lequel ledit chauffage est effectué par utilisation d'un rayonnement dans le proche infrarouge.

2. Procédé selon la revendication 1, dans lequel la vitesse de revêtement est d'au moins 350, de préférence au moins 400 m/min, plus particulièrement ne dépasse pas 700 m/min.

3. Procédé selon la revendication 1 ou 2, dans lequel ledit rayonnement infrarouge est émis à des températures dépassant 2500 K.

4. Procédé selon les revendications 1 à 3, dans lequel la feuille continue de papier de base est revêtue par extrusion sur les deux côtés.

5. Procédé selon les revendications 1 à 4, dans lequel ledit polymère est une polyoléfine, un polyacrylate ou un polyester.

6. Procédé selon les revendications 1 à 5, dans lequel ladite feuille continue de papier de base est préchauffée à une température comprise entre 30 et 125°C.

7. Procédé selon la revendication 6, dans lequel la température ne dépasse pas 90°C.

8. Procédé selon les revendications 1 à 7, dans lequel la feuille continue de papier de base est soumise à un ou plusieurs autres traitements additionnels, avant le revêtement par extrusion.

9. Procédé selon la revendication 8, dans lequel ledit autre traitement comprend au moins l'un parmi un traitement par décharge couronne, un traitement à l'ozone, un traitement à la flamme et un traitement au plasma.

10. Procédé selon les revendications 1 à 9, dans lequel le papier de base stratifié est un papier de base photographique stratifié avec un polymère.

11. Procédé selon la revendication 10, dans lequel le papier de base photographique stratifié avec un polymère est pourvu d'au moins une couche d'une émulsion photographique.

12. Procédé selon la revendication 11, dans lequel le papier de base photographique stratifié avec un polymère est pourvu d'au moins une couche formant sous-couche de gélatine entre le revêtement polymère et l'émulsion photographique.

13. Papier d'impression ou papier de base photographique stratifié avec un polymère comprenant une feuille continue de papier de base sur au moins un côté de laquelle est disposé un revêtement polymère en une quantité comprise entre 25 et 50 g/m², lequel papier stratifié peut être obtenu par le procédé des revendications 10 à 12.
